

## UNITED STATES PATENT OFFICE.

ELIAS BIELOUSS, OF WASHINGTON, DISTRICT OF COLUMBIA, ASSIGNOR TO HENRY A. GARDNER, OF WASHINGTON, DISTRICT OF COLUMBIA.

NITROCHLOR DERIVATIVES OF OPEN-CHAIN HYDROCARBONS AND PROCESS OF  
MAKING SAME.

No Drawing.

Application filed July 30, 1921. Serial No. 488,697.

To all whom it may concern:

Be it known that I, ELIAS BIELOUSS, a citizen of the United States, residing at Washington, in the District of Columbia, have invented certain new and useful Improvements in Nitrochlor Derivatives of Open-Chain Hydrocarbons and Processes of Making Same, of which the following is a specification.

10 This invention relates to certain novel products derivable from liquid or liquefiable hydrocarbons of the open-chain type by subjecting them or mixtures thereof to the successive steps of chlorination and nitration. With proper control of the process it is possible to obtain either solid or liquid nitro-chlor derivatives, both of these forms being usually produced simultaneously but in varying proportions according to the operating conditions. Both types of products possess properties indicating their applicability to numerous uses in the arts, for example as components of varnishes and of plastic molding compositions, and the like.

25 Only the lower members of the halogen-nitro-open-chain hydrocarbons have been heretofore known; and the principal methods for their preparation have involved the breaking down of hydrocarbon complexes, usually of the closed-chain type. A familiar example of this is the preparation of chloropicrin,  $CCl_3NO_2$ , which can be made either by the nitration of chloral or by the chlorination of picric acid. Nitro-chlor derivatives of aromatic hydrocarbons are on the contrary well known.

30 I have found that whereas the paraffins themselves are exceptionally indifferent to nitrating agents, they acquire a pronounced reactivity toward such agents by the previous introduction of chlorin into the chain. My novel process consists essentially therefore in subjecting to a nitrating process the chlorine derivatives of liquid or liquefiable 45 open-chain hydrocarbons.

The chlorination may be carried out in any of the well known ways, either with or without the addition of a catalyst, and need not therefore be further described. It has 50 been observed, however, contrary to expectation, that whereas hydrocarbon oils containing a limited chlorin content (say up to

20-25% chlorin based on the weight of the original oil) tend to yield a large proportion of solid resinous nitro-chlor derivatives, the 55 oils of decidedly higher chlorination (say 40-50% chlorin) tend to yield nitro-chlor derivatives which at ordinary temperatures may be regarded as heavy viscous liquids. The solid product, separated as far as practicable by centrifugalizing from the liquid appears initially as a yellow to brown powder, fusible at moderate temperatures up to about 110° C. or higher, soluble in a variety of solvents or solvent mixtures including 65 benzol, acetone, mixtures of benzol and alcohol, and the like. In particular, these nitro-chlor derivatives both of the liquid and solid types, possess the unusual property of being readily miscible with nitrocellulose 70 solutions, and may be compounded with nitrocellulose in the preparation of plastics. The solutions of the nitro-chlor derivatives, either with or without nitrocellulose, yield continuous varnish films on evaporation. 75

The nitration may be carried out in various ways, usually involving the use of sulfuric and nitric acids, or of sulfuric acid and a nitrate. For example the chlorinated hydrocarbons may be introduced directly 80 into the nitrating bath (sulfuric and nitric acids); or the chlorinated hydrocarbons may be first mixed with sulfuric acid and the nitric acid added to the mixture; or the chlorinated hydrocarbon may be mixed with 85 sodium nitrate and the mixture introduced into the sulfuric acid bath. The proportionate yield of the solid and liquid nitro-chlor derivatives will vary considerably according to the specific operating method 90 chosen.

*Example I.*

A paraffin type mineral oil distillate of specific gravity 0.882 was chlorinated until 95 17% of chlorin by weight of the oil had been absorbed. 100 parts by weight of this chlorinated oil were added in small portions with stirring to a nitrating bath containing: 360 parts of sulfuric acid (97%) 65 parts 100 of nitric acid (70%). The temperature was not permitted to rise above 55° C. After standing a few hours the nitro-chlor derivative was parted from the residual acid, and

the solid resin separated from the liquid by pressure filtration. The solid product was thoroughly washed with water and gasoline and dried at room temperature. Approximately 37 parts by weight of a yellow low-melting resin having the properties above described were obtained.

*Example II.*

10 100 parts of the above chlorinated oil were mixed with 360 parts of sulfuric acid (97%), and 65 parts of nitric acid (70%) were added to the mixture in small successive portions. After treating the reaction mixture 15 as above 50 parts of a dark yellow resin were recovered.

*Example III.*

10 100 parts of a chlorinated oil containing 18% of chlorin were mixed with 160 parts 20 of sulfuric acid (97%) and 65 parts of nitric acid (70%) were added in small successive portions to the mixture. The product 25 was treated as above and 46 parts of a brown resin were recovered.

*Example IV.*

100 parts of the above chlorinated oil 30 were mixed with 60 parts of sodium nitrate, and 80 parts of sulfuric acid were added to the mixture in small portions. About 25 parts of a brown resin were recovered.

The melting point of the solid nitro-chlor derivatives prepared as above ranged from 60°-108° C. Their average nitrogen content was approximately 3.4%.

The liquid products are also principally nitro-chlor derivatives, and apparently comprise both nitro-chlor derivatives of lower nitrogen content, and nitro-chlor derivatives of the lower-boiling components of the original oil.

I claim:

Process of making nitro-chlor derivatives of open-chain hydrocarbons comprising subjecting a paraffin type mineral oil distillate of a specific gravity of not less than 0.882 45 successively to chlorination and nitration.

In testimony whereof, I affix my signature.  
ELIAS BIELOUSS.